

## [54] COPPER-BASE ALLOY FOR HIGH PRECISION RESISTORS

[76] Inventors: **Boris Vladimirovich Blinov**, ulitsa Frunze 4 kv.5; **Vasily Valentinovich Kukhar**, 2 Murinsky proezd 15 kv. 34, both of Leningrad, U.S.S.R.

[22] Filed: **Sept. 20, 1973**

[21] Appl. No.: **399,119**

## Related U.S. Application Data

[63] Continuation-in-part of Ser. No. 77,014, Sept. 30, 1970, abandoned.

[52] U.S. Cl. .... **75/161**, 338/334

[51] Int. Cl. .... **C22c 9/00**, C22c 9/06, H01c 13/00

[58] Field of Search ..... 75/153, 161; 338/334

## [56] References Cited

## UNITED STATES PATENTS

|           |        |                 |          |
|-----------|--------|-----------------|----------|
| 2,466,202 | 4/1949 | Brenner .....   | 75/161 X |
| 3,451,808 | 6/1969 | Thielmann ..... | 75/153 X |

## OTHER PUBLICATIONS

Metals Transactions, Vol. 185, pp. 495-499, August 1949.

Primary Examiner—C. Lovell  
Attorney, Agent, or Firm—Waters, Roditi, Schwartz & Nissen

## [57] ABSTRACT

An alloy especially useful for high precision resistor material consists essentially of about 8 to about 14% (by weight) of manganese, about 6 to about 10% (by weight) of gallium, and the balance being copper. Small amounts of germanium, indium, nickel and/or aluminum may be present. The alloy is characterized by having in combination extremely low first and second temperature coefficients of resistivity, extremely low thermal EMF vs. copper, extremely high time stability of all properties, excellent workability and high corrosion resistance.

8 Claims, No Drawings

# COPPER-BASE ALLOY FOR HIGH PRECISION RESISTORS

## CROSS-RELATED APPLICATION

This application is a continuation-in-part of our earlier application, Ser. No. 77,014 filed Sept. 30, 1970 now abandoned.

## BACKGROUND OF THE INVENTION

The present invention relates to copper-base alloys and more particularly to alloys which are especially useful as high precision resistor material.

Such an alloy shall meet the following requirements:

1. Its resistivity shall be sufficiently high (not substantially lower than 30-35  $\mu$  Ohm·cm);
2. Its first and second temperature coefficients of resistivity (i.e. first and second derivatives of resistivity with respect to temperature) shall be as low as possible;
3. Its resistivity shall remain constant over a prolonged period of time;
4. Its thermal electromotive force (EMF) versus copper shall be as low as possible;
5. It shall possess a high degree of corrosion resistance in the operating temperature range;
6. Its workability shall be good enough to produce readily sufficiently fine wires, strips, ribbons etc.

Among the copper-base alloys known in the art the most suitable for use as a high precision resistor material are the following alloys:

(the symbol "%" below and throughout the specification and the claims means "weight %" unless otherwise specified)

a. Alloys known under the trademark "Manganin." Such alloys contain 2 to 4 percent nickel and 10 to 13 percent manganese, the remainder being copper. Manganin type alloys are disclosed e.g. in the "Alloy Digest," Filing Code Cu-126 and in U.S. Pat. No. 3,451,808 to Thielmann, lines 26 to 53 in the col. 1 and No. 1 alloy in the table on col. 3-4;

b. "Therlo" alloy comprising 5.5% aluminum, 9.5% manganese, the remainder being copper. This alloy is disclosed e.g. in NBS Circular 470, p. 4 (reprinted in vol. 3 of NBS Special publication 300, see p. 155), see also the above-mentioned U.S. Pat. to Thielmann, lines 54-63 in the col. 1;

c. Copper-manganese-germanium alloys comprising 6 to 22% manganese and 0.1 to 8% germanium optionally also small amounts of some other metals (tin to 3%, antimony to 1%, arsenic to 0.5%, gallium to 5%, indium to 1%, aluminum to 5%, zinc to 5%, nickel to 5%, all these metals together should not exceed about 10%), the remainder being copper. Such alloys are disclosed by Thielmann (U.S. Pat. No. 3,451,808, British patent specification No. 1,155,051 etc.) and by Hirayama (Japanese patent specifications No. 34-2407 and No. 37-11404 as well as his monograph published as No. 618 of the "Researches of the Electrotechnical laboratory" series, Tokyo, Oct. 1961, see especially p. 5 of the English "Synopsis" attached to this monograph).

However, none of the alloys known in the art do fully meet the above cited requirements.

The disadvantages of the previously known "Manganin" and "Therlo" alloys are described e.g. in the above-mentioned U.S. patent to Thielmann.

Copper-manganese-germanium alloys disclosed by Thielmann and by Hirayama also have appreciable disadvantages.

Such alloys with high germanium content (over 3 percent) while having good values of temperature stability of resistance, do not possess sufficient stability of electrical properties in time. Their thermal EMF vs. copper is relatively high. And — last but not least — such alloys cannot be readily worked, they are fragile, and forging of ingots to make rods etc. is inherently tied with considerable amount of waste. Nos. 3 and 4 alloys of the Thielmann patent, containing 6 and 8% of germanium respectively, are exemplary for such alloys. As may be seen from the table on col. 3-4 of the Thielmann patent, thermal EMF vs. copper is for each of these alloys about 2.5 times as high as that for "Manganin." Such relatively high values of thermal EMF vs. copper preclude the possibility of performing highest precision measurements with employment of resistors made from these alloys. It is worth noting also that if copper-base alloys have high thermal EMF vs. copper (as is the case for the alloys Nos. 3 and 4 of Thielmann patent) this indicates the appreciable discrepancy of Fermi levels (chemical potentials) for the alloy and for copper which in turn causes the instability of the alloy-copper system (e.g., instability of resistance of the whole resistor — leads — terminals system). A high germanium content in a copper-base alloy necessarily implies a relatively high thermal EMF of such alloy vs. copper (as is stated e.g. by Thielmann in the above-mentioned British patent specification No. 1,155,051, page 2, lines 5 to 9). In the above-mentioned Japanese patent specification No. 34-2407 it is explained (see page 2, left column, lines 1 to 3 and also page 2, right column, lines 7 to 13) that copper-manganese alloys with a germanium content higher than 3 percent show decomposition of solid solution, and, as a corollary, time instability and insufficient ductility. Therefore, the alloys with high germanium content, despite good temperature stability of their resistance, are apparently not very useful for making resistors of highest precision.

On the other hand, the resistivity of the copper-manganese-germanium alloys with low (under 3 percent) germanium content (e.g. of alloys Nos. 5 to 14 of the Thielmann patent and of the alloys disclosed in the above-mentioned Hirayama publications) is dependent in a much higher degree on the temperature. As may be seen from the drawing in the Thielmann patent, the resistivity variations in the temperature range 20° to 50°C are for alloys Nos. 5-14 within the limits 0.0025 to 0.008 percent. These limits are nearly 10 times worse than those for Thielmann alloys Nos. 3 and 4, while nearly 4 to 1.5 times better than those for "Manganin". The first temperature coefficient of resistivity  $\alpha_0$  for the alloys disclosed in the above-mentioned Japanese patent specification No. 34-2407 and in the Hirayama monograph is practically equal to zero, but the second temperature coefficient of resistivity  $\beta$  is not sufficiently low.  $\alpha_0$  and  $\beta$  are coefficients in the equation:

$$R_t = R_0(1 + \alpha_0(t - t_0) + \beta(t - t_0)^2)$$

where

65  $t_0$  is a standard or reference temperature (usually  $t_0 = 20^\circ\text{C}$  or  $t_0 = 25^\circ\text{C}$ )

$R_0$  is resistivity at temperature  $t_0$ , and

$R_t$  is resistivity at temperature  $t$ .

As stated by Hirayama, the  $\beta$  values for his alloys vary from  $-0.35 \cdot 10^{-6} \text{ }^{\circ}\text{C}^{-2}$  to  $-0.6 \cdot 10^{-6} \text{ }^{\circ}\text{C}^{-2}$ . It is highly desirable to reduce the  $\beta$  values even more. The lower the  $\beta$  value, the less the variation of resistivity in the same temperature range. Moreover, increasing the  $\beta$  values hardens the requirements for thermal treatment of alloy because variations in the thermal treatment result in shifting of the position of the upper point of the  $R-t$  curve, and the more flattened the curve, the less the effect of this shifting on the resistivity of the alloy at standard temperature  $t_0$ .

The resistance to corrosion and time stability for all the mentioned copper-manganese-germanium alloys are not fully satisfactory.

#### SUMMARY OF THE INVENTION

The present invention aims to avoid the above listed disadvantages of the alloys known in the art and to provide an alloy for highest precision resistors which will more fully meet the requirements for alloys of such a kind.

We have found that this aim may be achieved by providing copper-base alloys with manganese and gallium as two other main components. Most satisfactory properties are found in the copper-manganese-gallium alloys with 6% gallium or more.

Investigating the properties of ternary copper-manganese-gallium alloys has proved that the first temperature coefficient is equal to zero or very near it for alloys having a manganese content of 8.2 to 9 percent, the content of gallium being within the limits of about 3 to 10 percent. The temperature coefficient  $\beta$  is equal to 0 or very close to 0 for alloys having a manganese content of about 6 percent, the gallium content being equal to about 3 to 5 percent. If the gallium content is increased to exceed 5 or 6 percent, the amount of manganese required to obtain  $\beta = 0$  is gradually increased, and thus approaches the amount of manganese required to obtain  $\alpha = 0$ . This may be explained by the fact that exactly when the gallium content exceeds 5 to 6 percent in the alloy, a ternary intermetallic compound of copper, manganese, and gallium begins to be formed.

Small amounts of germanium, indium, nickel and/or aluminum (which will be referred to hereafter as secondary alloying metals) may be added. Most of the preferred embodiments of the proposed alloy may be described as an alloy substantially conforming to the stoichiometric formula  $\text{Cu}_5\text{Mn}$  with part of the manganese atoms (preferably not less than one third and not more than one half of the manganese atoms) substituted by gallium atoms or by gallium atoms and atoms of the mentioned secondary alloying metals (the amount of gallium atoms shall be not lower than the amount of atoms of the secondary alloying metals). In other words, the copper content shall be about 83.3 atomic percent, manganese content 8.3 to 11.1 atomic percent, gallium content 2.8 to 8.4 atomic percent, and the content of secondary alloying metals — up to 4.2 atomic percent. As we have found the copper content in such alloys does not exceed substantially 83-84 atomic percent if highest stability is required. However, the copper content may be a little lower, e.g. between 80 and 83 atomic percent. Both of the above-mentioned temperature coefficients of resistivity are very close to zero for the alloys according to the present invention.

The secondary alloying metals do not substantially affect the properties of the alloy. Germanium in an amount not exceeding 0.5 percent (by weight) serves as a deoxidizing agent and facilitates producing of sound castings and obtaining of desired component proportions. An addition of indium (not more than 1.5 percent) accelerates the process of alloy stabilization and enhances its corrosion resistance. Substituting a portion of gallium by aluminum reduces the cost of the alloy and increases its ultimate tensile strength. The addition of nickel further improves the corrosion resistance and also raises the tensile strength of the alloy, adding of aluminum and/or nickel do not cause appreciable worsening of the electrical properties of the alloy providing that the total amount of secondary alloying metals is not in excess of 5 percent.

It is therefore one object of the present invention to provide an improved alloy which is especially useful for highest precision resistors and possesses in combination the extremely low first and second temperature coefficients of resistivity, the extremely low thermal EMF vs. copper, high time stability, high corrosion resistance and good workability.

Another object of the present invention is to provide copper-base alloys for precision resistors containing 8 to 14 percent manganese, 6 to 10 percent gallium.

#### DETAILED DESCRIPTION OF PREFERRED EMBODIMENTS

Other objects of the present invention and advantageous features thereof will become apparent from the description.

The proposed alloy may preferably be produced by fusing the initial constituents in a crucible placed in a high frequency electric furnace under a protective layer of borax or in vacuum, or else, in an inert gas atmosphere, said crucible being made of alumina, with the subsequent casting of the product into copper molds. Wire and strip are produced from this alloy by plastic deformation. The alloy constituents preferably may be so selected as to correspond to stoichiometric formula of Kurnakov compound  $\text{Cu}_5\text{Mn}$ , wherein part of manganese is substituted by gallium or by gallium and at least one of the following secondary alloying metals: germanium (till 0.5% by weight), indium (till 1.5%), aluminum (till 5%) and nickel (till 5%). The total amount of the secondary alloying metals should not be in excess of 5 percent.

To make the present invention more fully apparent four alloy compositions are described below which are exemplary for our alloys.

The chemical composition of the alloys in Examples 1-3 is presented following the chemical analysis of the melt or a fresh cast ingot. The chemical composition of the alloy of Example 4 is presented following the chemical analysis of a wire made of the alloy. The chemical composition of the wire may slightly differ from that of the ingot it is made of, namely: the proportion of manganese in the wire may be by 0.2 to 0.5 percent lower than in the ingot, the content of the other elements being accordingly higher.

## EXAMPLE 1

An alloy containing 12% manganese, 6% gallium, 1% indium, 0.5% germanium, 80.5% copper (or, in atomic %, 13.9-5.5-0.5-0.4-79.7% respectively). The resistivity of this alloy is  $\rho = 50 \mu \text{ Ohm cm}$ , first and second temperature coefficients of resistivity are:

$$\alpha_{20} = -6 \cdot 10^{-6} \text{ }^{\circ}\text{C}^{-1}, \beta = -0.04 \cdot 10^{-6} \text{ }^{\circ}\text{C}^{-2};$$

thermal EMF vs. copper (in the 15° - 40°C temperature range)

$$\Delta E/\Delta t = -0.23 \mu \text{ V}/\text{C}$$

## EXAMPLE 2

An alloy containing 9% manganese, 6.6% gallium, 84.4% copper (or, in atomic %, 10.3-6.0-83.7% respectively) has the following electrical properties:

$$\rho = 36 \mu \text{ Ohm cm}, \alpha_{20} = 1.6 \cdot 10^{-6} \text{ }^{\circ}\text{C}^{-1}, \beta = -0.28 \cdot 10^{-6} \text{ }^{\circ}\text{C}^{-2}, \Delta E/\Delta t = -0.3 \mu \text{ V}/\text{C}.$$

## EXAMPLE 3

An alloy containing 9.2% manganese, 6.6% gallium, 0.2% germanium, 84% copper (or, in atomic %, 10.5 - 6.0 - 0.2 - 83.3% respectively). Electrical properties of this alloy are as follows:  $\rho = 37 \text{ Ohm cm}$ ,  $\alpha_{20} = 0.2 \cdot 10^{-6} \text{ }^{\circ}\text{C}^{-1}$ ,  $\beta = -0.27 \cdot 10^{-6} \text{ }^{\circ}\text{C}$ ,  $\Delta E/\Delta t = -0.3 \mu \text{ V}/\text{C}$ .

## EXAMPLE 4

An alloy containing 8.4% manganese, 9.8% gallium, 81.8% copper (in atomic % 9.7 - 8.9 - 81.4% respectively). This alloy has the following properties:

$$\rho = 40 \mu \text{ Ohm cm}, \alpha_{20} = 0.2 \cdot 10^{-6} \text{ }^{\circ}\text{C}^{-1}, \beta = 0.09 \cdot 10^{-6} \text{ }^{\circ}\text{C}^{-2}, \Delta E/\Delta t = -0.3 \mu \text{ V}/\text{C}.$$

Thus the resistivity of our alloys is substantially the same as that of the known alloys. Temperature stability of resistance is as good as that for alloys with high germanium content (Nos. 3 and 4 alloys of Thielmann patent; the disadvantages of these alloys are discussed above). The value of thermal EMF vs. copper is for our alloys considerably lower than that for these alloys and even than for all known in the art precision resistor alloys except "Therlo."

The resistivity of our alloys does not vary more than by  $1 \cdot 10^{-6}$  per year (by  $1 \cdot 10^{-4}$  percent) providing proper thermal treatment and artificial aging are carried out as is well known in the art.

Our alloys have good mechanical and technological properties and excellent workability. They may be readily forged without significant amount of waste. From these alloys may be readily produced the finest wires, ribbons, strips etc. Ultimate tensile strength is

440-460 N/mm<sup>2</sup>. Elongation of wire made from our alloys equals for 0.5 mm diameter wire 34 to 45%, for 25 microns diameter — 23-28 percent (for Manganin 30 and 15 percent respectively, for alloys with high germanium content not more than 10 percent for 25 microns diameter wire).

Corrosion resistance of our alloys is not lower than that of "Therlo" and considerably higher than corrosion resistance of "Manganin" and copper-manganese-germanium alloys.

We claim:

1. An alloy especially useful as material for precision resistors, said alloy consisting essentially of between about 8% and about 14% of manganese, between about 6% and about 10% of gallium, and the remainder being copper.

2. An alloy according to claim 1 wherein the copper content is about 84.4%, the manganese content about 9% and the gallium content about 6.6%.

20 3. An alloy according to claim 1 wherein the copper content is about 81.8%, the manganese content about 8.4% and the gallium content about 9.8%.

25 4. An alloy especially useful as material for precision resistors, said alloy containing between about 8% and about 14% manganese, between about 6% and about 10% gallium, and at least one of the following additional secondary alloying metals in the amounts as given:

|           | up to about (percent) |
|-----------|-----------------------|
| Germanium | 0.5                   |
| Indium    | 1.5                   |
| Aluminum  | 5                     |
| Nickel    | 5                     |

35 the total amounts of said secondary alloying metals not substantially exceeding 5 percent, and the remainder being copper.

40 5. An alloy according to claim 4, wherein the copper content is about 80.5%, the manganese content about 12%, the gallium content about 6%, the indium content about 1%, and the germanium content about 0.5%.

45 6. An alloy according to claim 4, wherein the copper content is about 84%, the manganese content about 9.2%, the gallium content about 6.6%, and the germanium content about 0.2%.

50 7. An alloy especially useful as material for precision resistors, said alloy conforming to the stoichiometric formula  $\text{Cu}_5\text{Mn}$  with not less than one third and not more than one half of the manganese atoms substituted by gallium atoms.

55 8. An alloy according to claim 7, wherein not more than one half of the gallium atoms are substituted by atoms of at least one of the following metals: germanium, indium, aluminum and nickel.

\* \* \* \* \*

UNITED STATES PATENT AND TRADEMARK OFFICE  
CERTIFICATE OF CORRECTION

PATENT NO. : 3,847,602

DATED : November 12, 1974

INVENTOR(S) : Boris Vladimirovich Blinov et al.

It is certified that error appears in the above-identified patent and that said Letters Patent are hereby corrected as shown below:

Cover page, in amend "proezd" to read:  
the heading,  
inventors: -- prospekt --  
(line 3)

Column 2, line 2 amend "Thielmannand" to read:  
-- Thielmann and --

Column 5, line 10 amend to read:  
--  $\Delta E/\Delta t = -0.023 \mu V/^\circ C$  --

Signed and Sealed this

*Fifth Day of September 1978*

[SEAL]

*Attest:*

RUTH C. MASON  
*Attesting Officer*

DONALD W. BANNER  
*Commissioner of Patents and Trademarks*